

May 15, 1945.

R. G. QUINN

2,376,083

OIL STOVE WICK

Filed Oct. 5, 1943



INVENTOR

ROBERT G. QUINN.

By Virgil C. Kline  
ATTORNEY

## UNITED STATES PATENT OFFICE

2,376,083

## OIL STOVE WICK

Robert G. Quinn, Bound Brook, N. J., assignor to  
Johns-Manville Corporation, New York, N. Y.,  
a corporation of New York

Application October 5, 1943, Serial No. 505,012

7 Claims. (Cl. 67—69)

This invention relates to wicks for oil stoves, and particularly to non-combustible asbestos fiber wicks suitable for use in the annular wick holders of blue flame oil stoves.

The efficiency of an oil stove wick is determined by the rate at which heat is developed by a flame supplied with liquid fuel by said wick, and by the length of time that said wick will stand up under full flame operation without substantial carbonizing and disintegration such as would seriously reduce its efficiency. The most efficient oil stove wicks now available are fabric wicks of woven asbestos or glass fibers. Another type of oil stove wick which is of common use consists of several plies of conventional chrysotile asbestos paper. While a wick of this kind is less expensive, it is no more economical since it has a much shorter operating life and a lower operating efficiency in comparison with a woven asbestos fabric wick. Conventional multi-ply asbestos paper wicks are also deficient in capillarity to such an extent that the time required to feed a unit volume of oil upwardly by capillary action through a unit length of wick to a combustion flame is much longer for a conventional multi-ply asbestos paper wick than for woven asbestos or glass fabric wicks.

Objects of the present invention are to provide a wick for oil stoves which is economical and efficient and which can be manufactured and transported as a flat sheet and readily shipped and inserted in an annular wick holder without tearing or fraying.

With the above objects in view, the invention consists in the improved oil stove burner wick which is hereinafter described and more particularly defined by the accompanying claims.

In the following description reference will be made to the attached drawing, in which:

Fig. 1 is a perspective view of a three ply asbestos paper wick in flat sheet form, with the individual plies stapled together at one end and spread apart at the other end to show the flexible paper sheets;

Fig. 3 is a sectional view taken on line 3—3 of Fig. 1; and

Fig. 2 is a perspective view of the wick of Fig. 1 after being curved to tubular shape to conform to an annular wick holder.

Multi-ply asbestos paper laminate wicks, in accordance with the present invention, preferably incorporate at least one inner core ply of asbestos paper having a high capillarity for oil and having a high resistance against disintegration or carbonizing when installed and operated for long periods in a blue flame oil stove. Essentially, the

invention is based on the discovery that a core ply paper of the indicated desirable properties should incorporate as its major constituent asbestos fibers of the amphibole group including amosite, tremolite, anthophyllite or crocidolite. Such amphibole fibers should be well cleaned and should have a size classification according to the Standard Quebec wet screen test of approximately 11 ounces out of a 16 ounce sample retained 10 on a 10 mesh screen, and 5 ounces passed through a 10 mesh screen. In the preferred wick construction the two outer plies are preferably made up of conventional chrysotile fiber paper, for the reason that this paper is stronger and denser and 15 provides a heat insulating shell of low capillarity for oil by means of which the core of the wick is shielded and insulated from the hot metal walls of the wick holder. Wicks of more than three plies are frequently desirable for higher capacity units, and there may be several inner or core 20 plies of amphibole asbestos fiber paper.

The particular wick construction which is illustrated in the drawing is a three ply laminate sheet 10 of which the central or core ply 12 comprises an oil absorbent, amosite fiber paper having a thickness of .020-.040 inch and weighing 5-10 lbs. per 100 sq. ft. In manufacturing the paper constituting the core and outer plies of the wick, it is advantageous to incorporate in the 25 fiber furnish about 3% of its weight of a binder such as oxidized starch gum or calcium silicate. The outer plies 14 of the wick are preferably conventional asbestos paper of about .02 inch thickness and weighing about 8 lbs. per 100 sq. ft.

30 In manufacturing the wicks, the outer and inner plies of asbestos paper are preferably assembled in flat sheet form, and are shipped and stored in this form. The individual sheets may be assembled into the laminate wick structure 35 and attached by spot gluing or by stitching or by beads of sodium silicate. The preferred method of attaching the sheets together is by means of one metal staple 18 disposed at one end of the wick parallel to a short edge thereof, in such 40 a way as to hold the individual sheets of the laminate structure together without interference with the operations of shaping the wick and of inserting the wick in the annular wick holder.

Comparative tests of the capillarity and of the 45 operating efficiency of a three ply asbestos paper laminate wick having an amphibole paper core, in comparison with conventional woven asbestos fabric wicks and with conventional three ply chrysotile asbestos paper laminate wicks, have demonstrated that the amphibole paper core wick

of the present invention has an initial capillarity for oil at least double that of the woven asbestos fabric wick, and much greater than the capillarity of a conventional three ply chrysotile paper laminate wick. When a wick of 11" x 1 $\frac{3}{4}$ " dimensions consisting of a core 12 of amosite fiber paper of 0.35 inch thickness, clamped between two outer sheets 14 of conventional chrysotile paper of .02 inch thickness, was inserted in the wick holder of a stove and immersed about  $\frac{3}{8}$  of an inch in the oil reservoir, its capillary action was found to be such that it could be initially ignited within about 30 seconds. Under the same test conditions a woven asbestos wick required about 70 seconds for initial ignition. The amosite paper core wick of the present invention will continue to feed fuel after ignition with an even blue flame, whereas it frequently requires at least  $\frac{1}{2}$  hour of operation to attain an even blue flame combustion when using a woven asbestos wick, or when using a conventional three ply chrysotile asbestos paper wick.

A three ply amosite paper core wick such as herein described has been found to operate satisfactorily over an operating life of 500 hours in a burner developing an even blue flame. At the end of this 500 hour test period the wick still retains ample mechanical strength to withstand normal handling, including removal and reinsertion in the annular wick holder. Conventional multi-ply asbestos paper wicks do not possess this long operating life, and are very much lower in their operating efficiency. An improved multi-ply amphibole paper wick such as herein described will exhibit a heat developing efficiency at least equal to that of a woven asbestos fabric wick of the same thickness, as has been determined by calorimeter tests. Such efficiency is very much greater than that of any conventional three ply chrysotile asbestos paper wick of the same dimensions.

The operating efficiency and capillarity of the amphibole paper core wicks herein described drop gradually as the operating life increases above about 100 hours. However, because of their relatively lower cost, and because they retain rela-

tively high efficiency over operating periods of 300 to 400 hours, they are much more economical than conventional oil burner wicks now available, including conventional woven asbestos and glass fabric wicks.

Since many variations may be made from the illustrative details given, without departing from the scope of the invention, it is intended that the invention should be limited only by the terms of the claims interpreted as broadly as consistent with novelty over the prior art:

What I claim is:

1. A wick for oil stoves comprising a multi-ply asbestos paper laminate at least one inner core 15 ply of which comprises a sheet of amphibole fiber paper of .020-.040 inch thickness and having a weight of 5-10 lbs. per 100 sq. ft.

2. A wick for oil stoves comprising a multi-ply asbestos paper laminate having at least one inner core 20 ply of greater thickness than the outer plies and which consists chiefly of amphibole asbestos fibers.

3. A wick for oil stoves comprising a multi-ply asbestos paper laminate, at least one inner core 25 ply of which comprises a sheet of amosite fiber paper of .020-.040 inch thickness having a weight of 5-10 lbs. per 100 sq. ft., said amosite paper core being lightly sized with about 3% by weight of oxidized starch gum.

4. A wick for oil stoves as defined in claim 2 in which the outer plies comprise chrysotile asbestos paper of greater density than that of the core ply.

5. A wick for oil stoves as defined in claim 2 in which the wick plies are fastened together by a single metal staple adjacent to and paralleling a short edge of the wick.

6. A wick for oil stoves comprising a multi-ply asbestos paper laminate having at least one inner core 30 ply which consists chiefly of amphibole asbestos fibers.

7. A wick for oil stoves comprising a multi-ply asbestos paper laminate having at least one inner core 35 ply which consists chiefly of amosite asbestos fibers.

ROBERT G. QUINN.